

1

3,014,852

**CADMUM PLATING COMPOSITIONS**

William F. Hamilton, Altadena, and Welton R. Burney, Jr., Northridge, Calif., assignors to Lockheed Aircraft Corporation, Burbank, Calif.  
No Drawing. Filed Aug. 26, 1957, Ser. No. 680,397  
11 Claims. (Cl. 204—50)

This invention relates to the electrodeposition of cadmium and relates more particularly to electroplating baths useful in the electroplating of cadmium on ferrous metals. A general and important object of the invention is to provide for the effective dense deposition of cadmium from aqueous alkaline cadmicyanides without hydrogen embrittlement of the articles being plated.

The copending application of William F. Hamilton et al., Serial Number 568,944, filed February 29, 1956, discloses aqueous cadmicyanide plating compositions for the non-embrittling cadmium plating of ferrous metals, and the like, which utilize, essentially, a high percentage of cadmium metal and a low percentage of free cyanide with nitrate ions included to prevent the formation of hydrogen at the cathode under ordinary operating conditions and thus effectively avoid embrittlement of the parts being plated. The high percentage of cadmium metal, the low percentage of free cyanide and the nitrate ions are all required for non-hydrogen embrittlement over the normal ranges of current densities encountered in cadmium plating bath operations. In the plating bath compositions of the copending application small amounts of soluble alkylamines are utilized to increase both the throwing power and the plating efficiency.

An important object of the present invention is to improve the throwing power of non-embrittling aqueous cadmium cyanide electroplating solutions of the general character disclosed in the aforementioned copending application. It has been found that the amines when employed as throwing power additives tend to evaporate from the solutions and since the relative proportion of the additive must be carefully and accurately maintained such evaporation may cause a poor distribution of the plate and a reduced overall plating efficiency. On the other hand, any substantial excess in the amount of the amine additive will cause the plated parts to become embrittled at the current densities normally employed in the bath. We have discovered that in such a solution of high cadmium metal content and low free cyanide content, containing nitrate ions, the addition of water soluble polyethylene glycols materially increases both the efficiency of the plating operation and the throwing power of the solution and the problem of appreciable evaporation of the additive is avoided. Thus when a current density of 72 amperes per square foot is employed the cathode efficiency (with regard to the deposition of the cadmium), of a typical non-embrittling plating solution of the character hereinabove referred to, is less than 20% whereas with the addition to the solution of only approximately 0.05% by weight of mixed polyethylene glycols this efficiency increases to over 80%.

The non-hydrogen embrittling aqueous cadmium cyanide electroplating solutions of this invention may be said to comprise, generally, a relatively high percentage of cadmium metal, a relatively low percentage of free cyanide, hydroxide, nitrate ions for preventing or reducing the formation of hydrogen at the cathode and a relatively small proportion of water soluble polyethylene glycols for increasing both the throwing power and the plating efficiency of the bath.

While the electroplating compositions of this invention are useful in the cadmium plating of various metals we will herein refer to the plating of ferrous alloys having high ultimate tensile strengths, for example in the

2

range of from 260,000 to 280,000 pounds per square inch. Such steels or alloys are frequently employed in the fabrication of aircraft parts and elements such as landing gear, fuel tank attachments, motor mounts, and the like. In practice the weight saving effected by the employment of such high strength ferrous alloys in the construction of an airplane, may amount to several hundred pounds in a given large airframe. The susceptibility of these high strength ferrous alloys to rusting is a marked disadvantage and wherever possible the parts or members constructed of such alloys are cadmium plated. The cadmium plating in addition to covering the exposed surfaces of the ferrous alloy members provides anodic protection against corrosion should the plating become marred or scratched. The cadmium plating of the steel in conventional cyanide solutions is usually attended by the evolution of hydrogen and the hydrogen acts to embrittle the steel. Detection of such hydrogen embrittlement cannot be effected without destruction of the part or article tested and it is, therefore, impossible to properly demonstrate whether embrittlement has adversely affected a given part prior to its actual incorporation in the airplane. Since hydrogen embrittlement is quite common and its detection is difficult, it is not uncommon for a part or member of high strength steel to unpredictably fail in service due to hydrogen embrittlement occasioned by the cadmium plating operations. The effective cadmium plating of steel parts without hydrogen embrittlement thereof is accordingly extremely important, especially where failure of an embrittled member or part may cause a fatal accident or disaster. The present invention is, therefore, directed to the electroplating of cadmium by means of solutions or compositions which avoid hydrogen embrittlement of the ferrous metal parts and yet obtain continuous adherent dense coatings of the cadmium metal regardless of the shape or contour of the parts plated. As above indicated, this is effected by incorporating small amounts of polyethylene glycol or mixed polyethylene glycols in solutions of high cadmium metal content, low free cyanide content and containing nitrate ions.

Another and important object of the invention is to provide cadmium plating solutions of the character mentioned having ample and effective throwing power to assure adequate deposition of the cadmium metal in crevices, in the roots of threads, and on other irregularities and surfaces that are normally difficult to plate and that might normally cause rough, discontinuous or irregular plating. A cadmium electroplating solution of high cadmium, low free cyanide content and containing nitrate ions normally has poor throwing power and low plating efficiency. We have discovered, however, that the incorporation of mixed polyethylene glycols in such a solution imparts good throwing power and high or effective plating efficiency to the solution to assure the deposition of the cadmium in the roots of threads and on other surfaces otherwise difficult to properly plate.

Under extremely good plating conditions a smooth symmetrical part devoid of corners, crevices, etc. may be effectively cadmium plated with the solutions of the invention without any hydrogen embrittlement and without incorporating polyethylene glycol. However, in actual practice in plating operations where the parts to be plated have threads, abrupt corners, or other surfaces difficult to plate, the current densities of the plating bath are, of necessity, inherently varied in the bath because of the function of the electrical resistance therein. We have discovered that by incorporating relatively small amounts of mixed polyethylene glycols the throwing power of the bath or solution is increased and automatically compensates for the necessarily varied current densities in the bath at the surfaces of the part being plated. Thus

the cadmium plating solutions of this invention incorporating the small proportion of the mixed polyethylene glycols have sufficient and effective throwing power and are adequately efficient to assure the proper deposition of the cadmium metal on the parts, irrespective of their shapes. It is, therefore, an objective to provide cadmium plating solutions of the character described having relatively small amounts of an additive in the nature of mixtures of glycols of different average molecular weights, that is, different degrees of polymerization, to assure proper effective plating at the various current densities that are of necessity present in cadmium plating baths.

Another object of our invention is to provide electroplating solutions of this class composed of readily available materials compatible with the ingredients now commonly employed in the cadmium plating art and which enable the plating operations to be successfully and expeditiously carried out without hydrogen embrittlement of the parts being plated.

In employing the present invention cadmium metal is plated from an aqueous cyanide solution containing a relatively high percentage of cadmium metal and a relatively low percentage of free cyanide with nitrate ions added to prevent the formation of hydrogen at the cathode under the ordinary plating conditions and thus effectively avoiding embrittlement of the parts being plated. Conventionally, the addition of even small amounts of nitrate ions to cadmicyanide plating baths is avoided since both the efficiency of the bath and the quality of the resultant plating are adversely affected thereby. In employing the plating solutions of the present invention however the decrease of the efficiency of the bath due to the nitrate is counteracted by the additive. Another commonly recognized disadvantage of a high cadmium, low free cyanide plating bath containing added nitrate is the marked reduction in throwing power which means that the solution will usually or often fail to properly deposit the cadmium metal in the roots of screw threads, in narrow crevices, and on other irregularities of the plated parts, and the sensitivity of the plating to the condition of the surfaces of the article is extremely critical. Thus slight films of surface oxide, almost imperceptible grease films, and the like, may make the deposited cadmium plating rough, irregular, or discontinuous. In accordance with the present invention this disadvantage of the high cadmium, low free cyanide baths containing the added nitrate is also avoided and practically eliminated by the inclusion and maintenance in the bath of a small amount of mixed water soluble polyethylene glycols. The polyethylene glycols increase both the throwing power and the efficiency of the solution, reduce the sensitivity of the plating to surface conditions of the plated part and impart improved plating characteristics to the bath or solution. Under typical operating conditions we have found that the inclusion of the polyethylene glycols having selected average molecular weights enables the production of excellent fine-grained cadmium plate from suitably formulated solutions at current densities varying from less than 20 to more than 100 amperes per square foot. Amperes per square foot is herein abbreviated "a.s.f."

The degree of polymerization of the ethylene glycols utilized in the plating baths has a pronounced effect on the cadmium deposition at different current densities. In general polyethylene glycols having average molecular weights up to approximately 500 are most effective in producing improved plate at current densities exceeding about 100 a.s.f. while polyethylene glycols having average molecular weights in the range of from about 500 to about 1000 are most effective in the intermediate density ranges of from 50 to 100 a.s.f. and where the average molecular weights of the polyethylene glycols are between approximately 1000 and 1500 the most pronounced effect in increased throwing power and plating efficiency is with the lower current plating density ranges, for example up to approximately 50 a.s.f.

For good results under normal plating conditions with

the high cadmium metal, low free cyanide and nitrate bath, approximately 0.066 ounce per gallon of mixed polyethylene glycols may be employed. In such a case the polyethylene glycols may comprise a mixture of about 40% by weight having average molecular weights up to 500, about 40% by weight having average molecular weights between 500 and 1000 and about 20% by weight polyethylene glycols having average molecular weights between 1000 and 1500. We have found that when a total of less than 0.027 ounce per gallon of such a mixture of the soluble polyethylene glycols is used, the bath has a lowered plating efficiency and a reduced throwing or covering power. Where the proportion of the mixed polyethylene glycols is appreciably above 0.066 ounce per gallon the increase in plating efficiency and throwing or covering power is relatively small and unimportant. If a total concentration of the mixed polyethylene glycols is over about 0.13 ounce per gallon a slight permanent precipitate may appear in the bath since the limit of solubility of some of the higher molecular weight polyglycols may have been exceeded. Such a precipitate should be removed by filtration to avoid the formation of spots or stains on the cadmium plate.

The relative proportions of the several ingredients making up the improved electroplating baths of this invention are, of course, subject to considerable variation without bringing about hydrogen embrittlement of the ferrous metal parts being plated while employing normal ranges of current densities as conventionally utilized in such plating operations. We have found it is most desirable to maintain the nitrate content of the baths expressed in terms of sodium nitrate between approximately 3 and 28 ounces per gallon of the plating solution. The total cadmium metal content of the plating solution should preferably be between approximately 14 and 18 ounces per gallon. It has been noted that if the cadmium metal content is excessively low, hydrogen embrittlement of the plated metal may be encountered while if the cadmium metal content is excessively high, precipitation may result. While we have above referred to the nitrate content of the bath being expressed in the terms of sodium nitrate it is to be understood that nitrate ions may be incorporated in the solutions in other manners. For example, nitrate ions may also be added to the bath in the form of cadmium nitrate, thus simultaneously increasing the cadmium metal content of the solution. The nitrate ions may be added in whole or in part as sodium nitrate. In the plating solutions the nitrate ion is in a very alkaline medium and is normally surrounded by a stoichiometric excess of sodium ions so that it may be considered as existing as sodium nitrate in the solution for all practical purposes. Thus it will be seen that the addition of nitrate ions as sodium nitrate has substantially the same effect as introducing the ions in other forms.

It has been found that where the bath or plating solution contains about 16 ounces per gallon cadmium metal the total cyanide content in terms of sodium cyanide should be between 20 and 25 ounces per gallon and preferably about 22-23. The free sodium cyanide present in the plating solution determines the rate of increase of cadmium metal and the total cyanide present governs the total amount of the metal in the solution. In the event the free sodium cyanide exceeds about 4.00 ounces per gallon of the solution hydrogen embrittlement of the ferrous metal being plated may be induced due to decreased efficiency of the bath whereas if the free cyanide content of the solution falls below, say, 0.7 ounce per gallon the quality of the plating may be adversely affected.

As the plating operation progresses the sodium nitrate is gradually reduced to sodium nitrite and in order to prevent hydrogen embrittlement of the ferrous metal parts being plated due to local depletion of the nitrate constant agitation of the bath is important. It is preferred to maintain the sodium hydroxide content of the plating bath between approximately 5 and 10 ounces per

gallon. However the concentration of the sodium hydroxide is not believed to be critical. The percentage or concentration of the carbonate present in the solution is also relatively unimportant but in the event it builds up to an excessive value it may be removed by chilling and filtering the solution or by precipitation as an insoluble carbonate.

The following are typical preferred formulations for the electroplating baths or solutions of the invention from which it will be seen that substantial variation may be made without departing from the spirit of the invention.

*Example 1*

Prepare a solution as follows:

|                            | Ounces per gallon |
|----------------------------|-------------------|
| Sodium cyanide             | 27.3              |
| Cadmium oxide              | 15.2              |
| Sodium hydroxide           | 2.7               |
| Sodium nitrate             | 9.3               |
| Mixed polyethylene glycols | 0.054             |

The mixed polyethylene glycols are prepared by mixing equal parts by weight of polyethylene glycols with average molecular weights approximating 300, 400, 600 and 1000 and 1500 respectively and then warming the resultant mixture until a clear solution is obtained. The ingredients in Example 1 should be dissolved in distilled or de-ionized water in the order set forth. During use of the plating bath the solution should be controlled to remain within the following approximate limits by analysis:

|                      | Ounces per gallon |
|----------------------|-------------------|
| Total sodium cyanide | 20 to 25          |
| Free sodium cyanide  | 0.7 to 4          |
| Cadmium              | 14 to 18          |
| Sodium nitrate       | 3 to 28           |
| Sodium hydroxide     | 5 to 10           |
| Sodium carbonate     | A trace to 8      |

As the cadmium plating operation proceeds the content or proportion of the mixed polyethylene glycols should be controlled by making comparative tests in a "Hull" cell and preferably in no event should exceed a total concentration of about 0.1% by weight (0.13 ounce per gallon) or fall below a total concentration of 0.02% by weight (0.026 ounce per gallon).

*Example 2*

A cadmium plating solution containing about 10% cadmium metal in sodium cyanide may be prepared as follows:

|                | Ounces |
|----------------|--------|
| Sodium cyanide | 22     |
| Cadmium oxide  | 15     |

In preparing the bath of Example 2 the sodium cyanide is dissolved in about one-half gallon of distilled or de-ionized water and the cadmium oxide is then slowly added to the solution which is stirred continuously until the cadmium oxide is completely dissolved. 7.8 ounces of potassium nitrate is then added to the solution and water is added to bring the volume to approximately one gallon. The throwing power and efficiency increasing additive is then incorporated by adding two milliliters of polyethylene glycol having an average molecular weight of approximately 400 and one milliliter of polyethylene glycol with an average molecular weight of approximately 1000.

*Example 3*

In about 3 quarts of distilled or de-ionized water dissolve 14.5 ounces of cadmium nitrate tetra hydrate. Then add 26.6 ounces sodium cyanide and after it has been slowly dissolved add 17.7 ounces cadmium oxide and stir until the solution clears. Then after adding and dissolving 2.6 ounces sodium hydroxide make the solution to a volume of one (1) gallon by the addition of water.

With the addition of 0.03 ounce of polyethylene glycol

having an average molecular weight of about 600 this solution will plate cadmium metal satisfactorily under ordinary plating conditions and with the current density of 100 a.s.f. or more without noticeable hydrogen embrittlement.

*Example 4*

In about 4 gallons of distilled or de-ionized water dissolve:

|    |                                                                                    |             |      |
|----|------------------------------------------------------------------------------------|-------------|------|
| 10 | Sodium cyanide                                                                     | -----pounds | 9    |
|    | Cadmium oxide                                                                      | -----do     | 5    |
|    | Sodium nitrate                                                                     | -----do     | 6.6  |
|    | Polyethylene glycol having an average molecular weight of 400                      | -----ounces | 0.15 |
| 15 | Increase the final volume to 5.25 gallons by adding distilled or de-ionized water. |             |      |

This solution of Example 4 will plate cadmium metal on steel without visible cathodic gassing or without embrittlement with a current density from as low as about 20 a.s.f. to as high as about 100 a.s.f. Note that Example 4 contains a polyethylene glycol additive of a given or relatively narrow molecular weight range. A bath or solution containing such an additive may be used successfully where the parts to be plated are symmetrical or relatively symmetrical so that the inherent electrical resistances present in the bath are generally uniform.

It is of importance that the surfaces of the articles to be plated are properly prepared. All grease, oil, and surface films should be removed before the articles are immersed in the plating bath. The plating bath or solution should be continuously agitated and the cathodic articles kept in motion to prevent local depletion of the bath or changes in the concentration of its components.

35 High strength steel parts or articles may be effectively plated in the baths of our invention without the visible evolution of gas at the cathode and without noticeable hydrogen embrittlement.

The baths or solutions may be maintained in operative condition by the usual methods well known to those skilled in the art. An excessive increase or build up of sodium carbonate may be reduced by chilling the solution to about 50° F. and decanting or filtering. Alternately a solution of barium nitrate may be added, for example, to

45 decrease the carbonate by precipitating it as barium carbonate and simultaneously increasing the sodium nitrate content of the solution by double decomposition. As above pointed out, nitrate ions may be added to the bath in the form of cadmium nitrate thus simultaneously in-

50 creasing the cadmium metal content of the solution. In the event the plating solutions contain an excessive amount of cadmium hydroxide nitrate ions may be added as nitric acid. This should be done very slowly and with rapid stirring and extreme caution as the reaction of the

55 acid is violent and the hydrogen cyanide is toxic. The resulting sodium nitrate is neutral and the amount of free alkali is thus decreased. Higher proportions or concentrations of nitrate, approaching its limit of solubility, in the baths tend to prevent "burning" of the plate at the higher

60 current densities and do not appear to cause any salient untoward effects.

It is to be understood that our invention is not to be construed as based upon or dependent upon any theories which we have expressed. Nor is the invention to be regarded as limited to the express procedures or materials set forth, these details being given only by way of illustration and to aid in clarifying the invention. We do not regard such specific details as essential to the invention except insofar as they are expressed by way of limitation in

70 the following claims wherein it is our intention to claim all novelty inherent in the invention as broadly as permissible in view of the prior art.

We claim:

1. A non-embrittling cadmicyanide electroplating solution comprising from approximately 14 to approximately

18 ounces per gallon cadmium metal, from approximately 0.7 to approximately 4 ounces per gallon free sodium cyanide, from approximately 3 to approximately 28 ounces per gallon alkali metal nitrate, and from about 0.027 to about 0.13 ounce per gallon of water soluble mixed polyethylene glycols having different average molecular weights ranging between approximately 300 and 1500.

2. A non-embrittling cadmicyanide electroplating solution comprising from approximately 14 to approximately 18 ounces per gallon cadmium metal, from approximately 0.7 to approximately 4 ounces per gallon free sodium cyanide, from approximately 3 to approximately 28 ounces per gallon alkali metal nitrate, and from about 0.027 to about 0.13 ounce per gallon of water soluble mixed polyethylene glycols having different average molecular weights ranging from 300 to 1500.

3. A non-embrittling cadmicyanide electroplating solution comprising from approximately 14 to approximately 18 ounces per gallon cadmium metal, from approximately 3 to approximately 28 ounces per gallon alkali metal nitrate, and from 0.027 to about 0.13 ounce per gallon of water soluble mixed polyethylene glycols having different average molecular weights ranging between approximately 300 to 1500.

4. A non-embrittling cadmicyanide electroplating solution comprising from approximately 14 to approximately 18 ounces per gallon cadmium metal, from approximately 3 to approximately 28 ounces per gallon alkali metal nitrate, and from 0.027 to 0.13 ounce per gallon of water soluble mixed polyethylene glycols having different average molecular weights ranging from about 300 to about 1500.

5. An aqueous electroplating bath containing in terms of ounces per gallon, from 20 to 25 ounces sodium cyanide, from 14 to 18 ounces cadmium, from 3 to 28 ounces sodium nitrate, from 5 to 10 ounces sodium hydroxide, and about 0.05 ounce mixed water soluble polyethylene glycols having different average molecular weights ranging from 300 to 1500.

6. An aqueous electroplating bath containing in terms of ounces per gallon, about 27 ounces sodium cyanide, about 15 ounces cadmium oxide, about 3 ounces sodium hydroxide, about 9 ounces sodium nitrate, and about 0.05 ounce polyethylene glycol having an average molecular weight ranging between approximately 300 and 1500.

7. An aqueous electroplating bath containing in terms of ounces per gallon, about 27 ounces sodium cyanide, about 15 ounces cadmium oxide, about 3 ounces sodium hydroxide, about 9 ounces sodium nitrate, and from 0.027 to about 0.13 ounce mixed polyethylene glycols having

different average molecular weights ranging from 300 to 1500.

8. An aqueous electroplating bath containing in terms of ounces per gallon, about 27 ounces sodium cyanide, about 15 ounces cadmium oxide, about 3 ounces sodium hydroxide, about 9 ounces sodium nitrate, and from about 0.027 to about 0.13 ounce of substantially equal parts by weight of mixed polyethylene glycols having different average molecular weights of approximately 300, 600, 1000 and 1500 respectively.

9. An electroplating solution containing about 1 gallon water, about 14.5 ounces cadmium nitrate tetrahydrate, about 26.6 ounces sodium cyanide, about 17.7 ounces cadmium oxide, about 2.6 ounces sodium hydroxide, and about 0.03 ounce polyethylene glycol having an average molecular weight of about 600.

10. An electroplating solution comprising approximately 5.25 gallons water, 9 pounds sodium cyanide, 5 pounds cadmium oxide, 6.6 pounds sodium nitrate, and 0.15 ounce polyethylene glycol having an average molecular weight of about 400.

11. A non-embrittling cadmicyanide electroplating solution comprising from approximately 14 to approximately 18 ounces per gallon cadmium metal, from approximately 0.7 to approximately 4 ounces per gallon free sodium cyanide, from approximately 3 to approximately 28 ounces per gallon alkali metal nitrate, and from about 0.027 to about 0.13 ounce per gallon of water soluble mixed polyethylene glycols having different average molecular weights ranging from 300 to 1500 comprising about 40% by weight polyethylene glycols having an average molecular weight up to 500, about 40% polyethylene glycol having average molecular weights between 500 and 1000 and about 20% by weight polyethylene glycols having average molecular weights between 1000 and 1500.

#### References Cited in the file of this patent

#### UNITED STATES PATENTS

|    |           |                        |               |
|----|-----------|------------------------|---------------|
| 40 | 2,107,806 | Soderberg et al. ----- | Feb. 8, 1938  |
|    | 2,848,393 | Foulke et al. -----    | Aug. 19, 1958 |
|    | 2,881,121 | Foulke et al. -----    | Apr. 7, 1959  |
|    | 2,892,761 | Hamilton et al. -----  | June 30, 1959 |

#### FOREIGN PATENTS

|    |         |              |               |
|----|---------|--------------|---------------|
| 45 | 464,545 | Canada ----- | Apr. 18, 1950 |
|----|---------|--------------|---------------|

#### OTHER REFERENCES

Flora: American Journal of Science, vol. 20 (1905),  
50 pp. 454-455.